

April 5, 1955

DE WITT R. PETTERSON  
LATERALLY EXTENSIBLE POLYORIENTED NONWOVEN  
FABRIC AND METHOD OF PRODUCING SAME  
Filed April 7, 1952

2,705,692

2 Sheets-Sheet 1



INVENTOR  
DE WITT R. PETTERSON.

BY  
Benton A. Buee  
ATTORNEY

April 5, 1955

DE WITT R. PETTERSON  
LATERALLY EXTENSIBLE POLYORIENTED NONWOVEN  
FABRIC AND METHOD OF PRODUCING SAME  
Filed April 7, 1952

2,705,692

2 Sheets-Sheet 2

Fig. 7.



Fig. 8.



Fig. 9.



Fig. 10.



INVENTOR  
DE WITT R. PETTERSON  
BY  
Benton A. Bue  
ATTORNEY

# United States Patent Office

2,705,692

Patented Apr. 5, 1955

1

2,705,692

## LATERALLY EXTENSIBLE POLYORIENTED NON-WOVEN FABRIC AND METHOD OF PRODUCING SAME

De Witt R. Peterson, West Springfield, Mass., assignor to Chicopee Manufacturing Corporation, a corporation of Massachusetts

Application April 7, 1952, Serial No. 280,968

17 Claims. (Cl. 154—101)

The present invention relates to textile fabrics, and more particularly to so-called "nonwoven" fabrics produced from unspun textile fibers without the use of conventional weaving or knitting operations. The invention is of primary importance in connection with (and represents an improvement over) "oriented" nonwoven fabrics composed of textile fibers that are substantially oriented or "parallelized" in one direction.

Nonwoven fabrics are conventionally manufactured by producing an oriented web or sheet of loosely associated textile fibers (using any one of a variety of well-known procedures) and then converting the web into a conventional base web for such fabrics is produced continuously by a cotton card machine with the fibers substantially parallelized or oriented in the "machine direction," i. e., in the direction in which the product moves continuously from the sheet-forming machine.

The bonding operation by which such a web is converted into a fabric may be accomplished in one of several different ways. One way is to impregnate the web over its entire width with various well-known bonding agents such as natural or synthetic resins. Another method is to imprint on the webs a series of spaced, straight or wavy lines of binder extending continuously across the web. A more recent innovation (hereinafter referred to as "island bonding") involves imprinting on the web a discontinuous binder pattern comprising discrete areas or "islands" of binder arranged in overlapping columns parallel to each other and to the direction of fiber orientation, to form a uniform, staggered pattern such that every line within the overlap zone formed by the overlapping columns that is parallel to the direction of fiber orientation passes through at least three discrete binder areas within a distance along said line equal to the average length of the fibers comprising the web.

Where the individual "islands" are physically separated from each other by an appreciable distance but are nevertheless hingedly interconnected by bands of unbonded lengths of fibers, with the binder covering only a minor proportion of the lateral surface of the web, desirable textile-like properties are obtainable in the fabric, together with a number of interesting and important physical properties, the nature and degree of which are dependent in part upon the particular binder geometry employed. If the individual binder areas or "islands" are substantially symmetrical and the lateral surface covered by the binder areas does not substantially exceed about 35% of the total lateral surface of the web, the fabric is characterized by a pronounced capacity for lateral extension when the fabric is stressed in the cross direction. A fabric of this type wherein the binder areas are annular or ringlike in configuration is characterized by lateral extensibility to an outstanding degree.

When an island bonded web of high lateral extensibility is stretched cross wise, it expands on the "lazy tongs" principle with a major reorientation of the originally parallelized fibers, and the formation of a net-like or reticular structure. This reorientation is accompanied by what may be termed a "serpentine effect," i. e., with the generation of a series of parallel, sinuous or serpentine bands of fibers each band being the substantial reflection or mirror image of adjacent bands on either side with the bands united into a reticular structure by binder areas located at their points of apposition. Dimensional stability may be given to the resulting

2

stretched fabric by rebonding it in its laterally extended condition. Depending in part on the degree to which the basic fabric was stretched before rebonding, the ratio of long strength to cross strength of the resulting fabric differs markedly from the corresponding ratio of the fabric from which it was made. Indeed, if the basic or starting fabric is stretched to a substantial degree (e. g., 170% of its original width) before rebonding, the normal ratio of long-to-cross tensile strength may actually be reversed. It is thus possible to convert a non-isotropic, oriented fabric into a "pseudo-isotropic" fabric, whose cross strength equals or exceeds its long strength, a substantial proportion of the fibers being reoriented into a multiplicity of substantially sinuous or serpentine bands.

In a laterally extensible, island bonded fabric of the foregoing type, the binder areas constitute, in effect, the pivotal points of the "lazy tong parallelograms," while the bands of fibers connecting the pivotal points form the four sides of the collapsible parallelograms. Due to the far greater strength of the fiber bands relative to that of the binder areas which hold the serpentine bands together at their apposition points, the resin areas, even when reinforced by randomly disposed fibers located in such areas, represent the weakest points in the "lazy tong parallelograms." In such fabrics, rupture is therefore most apt to occur at the locus of the binder areas.

The broad object of the present invention is to provide a nonwoven fabric characterized by essentially the same lateral extensibility on the "lazy tongs" principle but by inherently greater strength and tear resistance compared to prior fabrics of this general type.

Another object is the provision of a "bias lay" nonwoven fabric whose structure and appearance resemble those of a woven fabric cut on the bias.

A further object is to provide means whereby the inherent tensile strength of the fibers may be utilized to a substantially greater degree in producing a nonwoven fabric that is laterally extensible on the lazy tongs principle.

Another object is a nonwoven fabric of the character described wherein substantially more fibers are utilized in the lazy tong structure.

A still further object is to provide a nonwoven fabric that is inherently stronger and more resistant to tear than a similar nonwoven fabric which undergoes reorientation with the "serpentine action."

A more specific object is to provide a fabric of the character described wherein the pivotal points of the "lazy tongs" are inherently the strongest "links" of the fabric, being formed, not by discrete binder areas joining separated sinuous fiber bands at their points of apposition, but by binder areas joining intersecting fiber bands at their points of intersection and therefore reinforced by the intersecting fibers of the respective bands.

Another object is a nonwoven fabric capable of elongation in either the long or cross direction, within controllable degrees.

Still another object is to provide means by which to reduce the degree of cross-drafting that is necessary in order to reverse the normal long-to-cross tensile strength ratio in the manufacture of a pseudo-isotropic nonwoven fabric by cross-drafting a prebonded nonwoven fabric and then rebonding the stretched fabric in its extended condition.

A further object is an improved "pseudo cross-lay" laminated fabric made from the pseudo-isotropic product described above.

Another object is to provide a simple method for producing fabrics of the foregoing type.

Other objects and advantages of the present invention will become apparent as the description progresses in connection with the several figures of the drawing which illustrate the preferred embodiments of the invention and the manner in which it may be carried into practice. In such drawings:

Figs. 1, 3 and 5 are, respectively, plan views of fragments of three different fabrics made from a two-ply "di-oriented" base web bonded in accordance with one embodiment of the invention, the fabrics being in their relaxed unextended state;

Figs. 2, 4 and 6 are plan views of the fabrics of Figs.

1, 3 and 5, respectively, the fabrics being in their extended or stretched condition;

Figs. 7 and 9 are, respectively, plan views of fragments of two different fabrics made from a three-ply "tri-oriented" base web bonded in accordance with the present invention;

Figs. 8 and 10 are plan views of fragments of the fabric of Figs. 7 and 9, respectively, the fabrics being in their extended or stretched condition.

Referring now particularly to Figs. 1 and 2 of the drawing, one embodiment of the invention comprises two series of parallel, substantially straight bands of fibers, generally indicated by the reference characters 10, 12, 14, 16 and 18. Each band in each series is composed predominantly of substantially parallelized, unspun textile fibers (e. g., 20) that are oriented with the axis of the band in which they lie. The two series of parallel bands are obliquely disposed with respect to each other at the angles  $\alpha$  and  $\beta$  from the horizontal, so that the bands of one series obliquely intersect the bands of the other series. The intersecting bands are held together at their points of intersection by discrete areas of binder (22, 24, 26, 28, 30, 32, 34 and 36) infused locally into the body of the bands at selected points of intersection. Preferably a multiplicity of unspun and unbonded (i. e., "free") textile fibers (e. g., 38 and 40) are disposed between, and substantially oriented with, each pair of the bands in each of the two series.

The resulting fabric may be likened to a collapsible "lazy tong" gate in its partly unextended or collapsed condition, the intersecting bands of fibers acting as linkages of the gate, the binder areas at selected points of intersection forming the pivotal points of the "lazy tong." In any event, regardless of the aptness or inaptness of the analogy suggested, the resulting fabric is laterally extensible when subjected to extensional stress in a direction parallel to either axis of the parallelograms formed by the intersection of the two series of parallel fiber bands. In the extended condition, the fabric of Fig. 1 assumes the condition shown in Fig. 2.

A modification of the fabric of Figs. 1 and 2 is shown in Figs. 3 and 4. In this case the binder areas, generally indicated by the reference character 42, are arranged in parallel courses (extending horizontally across the page) and also in parallel but non-overlapping columns (extending vertically on the page). The net effect of this "nonstaggered" arrangement of binder areas is a pair of "lazy tong" mechanisms, the pivotal points of one of the pairs (e. g. 44) being disposed in the centers of the parallelograms of the other (e. g. 46, 48, 50, 52).

In Figs. 5 and 6, another modification is shown. In this case the binder areas are arranged in staggered courses, as in Figs. 1 and 2, but are much closer together so that the net effect is a series of three lazy tong mechanisms, the pivotal points (e. g., 54 and 56) of two of them being disposed in the parallelograms of the third (e. g., 58, 60, 62 and 64).

From a comparison of the three fabrics illustrated in Figs. 1-6, it will be apparent that the fabric of Figs. 1 and 2 will have the greatest amount of free fiber between the fiber bands forming the parallelograms, while the fabric of Figs. 5 and 6 will have the least free fiber. The fabric of Figs. 3 and 4 will, of course, have an intermediate amount of free fiber.

It will also be apparent from inspection of Figs. 1 to 6 that the basic web from which these three embodiments are made comprises a sheet of loosely associated textile fibers that are predominantly oriented in two principal directions, one of the primary directions of orientation being obliquely disposed with respect to the other. Thus the basic web utilized in these examples may be termed a "di-oriented" web, i. e., a web having two primary axes of orientation as indicated by the arrows in Figs. 1 to 6.

One method of forming such a di-oriented web is simply to ply together two webs each consisting of substantially oriented textile fibers, with their respective axes of orientation obliquely disposed with respect to each other; the bonded di-oriented web may therefore be termed a "bias lay" fabric as distinguished from a "cross lay" fabric. The smaller of the two pairs of angles formed by the intersection of the respective axes of orientation of the two plies may lie between, say, 10° and 80°. Preferably, however, the angle ( $\alpha$ ) between the orientation axes of the respective webs should be in the

lower range of, say, 10° to 45°, corresponding to the angular relation of the linkages in a collapsible gate in its relatively unextended or collapsed condition; this gives the fabric greater capacity for lateral extension. The proportion of oriented fibers in the individual plies may vary within wide limits ranging from about 75% (as in a normal card web that has not been drafted and is not under tension) to as high as about 95 to 100% (as in the case of a highly drafted card web maintained in a state of tension in the long direction).

Referring now to Figs. 7 to 10, the base web in these examples is a "tri-oriented web," formed, for example, by plying together three different plies, each ply being substantially oriented in a given direction, the orientation direction of each ply being obliquely disposed with respect to the orientation directions of the other two plies. In such a "tri-oriented" web, interesting fiber reorientation effects are obtainable upon cross drafting after island bonding. The nature of these effects will depend in part upon the geometry of the binder pattern, particularly on whether the parallel columns of binder areas (i. e., vertically on the page of the drawing) are overlapping or nonoverlapping with respect to each other.

In Figs. 7 and 8, the individual binder areas 72, 74, 76, 78, 80, 82, and 84 are annular in configuration and are arranged in parallel, nonoverlapping courses (i. e., horizontally on the page) and also in parallel, nonoverlapping columns (i. e., vertically on the page). The fiber orientations are indicated by the three crossed arrows. When the fabric of Fig. 7 is stretched in the direction generally across the three axes of orientations, the fabric exhibits the same lazy tong action as in the case of the fabrics of Figs. 1 to 6 that were made from the di-oriented webs, assuming the condition shown in Fig. 8. In addition, the fabric of Fig. 7, upon cross drafting to form the fabric of Fig. 8 develops "puckered" fibers 86, i. e., fibers that are bent out of the plane of the fabric proper. These puckered fibers originate in part with the fibers which originally were oriented in the vertical direction and which connect binder areas in the same column (e. g., 72, 76 and 80).

In Figs. 8 and 9, the base web again consists of a tri-oriented web, formed, for example, from three plies, each ply being substantially oriented in a given direction, each orientation direction being oblique with respect to the orientation directions of the other two webs, as indicated in the three crossed arrows. However, in this example the individual binder areas are arranged in parallel nonoverlapping courses, and in parallel but overlapping columns. When the fabric of Fig. 8 is stretched crosswise, the collapse of the lazy tong structure produces not only "free fibers" 90 and "puckered fibers" 92, but also "serpentine fibers" 94 and 96. The latter or serpentine fibers were generated by the "serpentine effect" from the fibers that originally were oriented in the vertical direction and lay in the overlapping zone of the overlapping vertical columns, connecting opposite sides of adjacent resin areas (e. g., 72, 74, 76) in overlapping columns. Thus, the lazy tongs formed by coaction of the serpentine bands with the resin areas located at their points of apposition, are reinforced by lazy tongs formed by intersecting, substantially straight bands of parallelized fibers bonded together at their points of intersection.

It will thus be apparent that the nonwoven fabric of the present invention comprises an island bonded web composed of two or more plies of oriented fibers, the directions of orientation of the respective plies being inclined obliquely with respect to each other. The multi-ply web is bonded into a self-sustaining fabric by discrete areas of binder infused locally into the body of the web at selected, uniformly spaced points of intersection of the fibers. The binder areas coact with the oriented fibers in each ply to form a plurality of interconnected collapsible polygons, whose pivotal points are the discrete binder areas and whose sides consist of bundles of substantially parallel, straight (nonsinuous) fiber bands connecting the binder areas.

The base web may consist of either two or more plies. Where the base web consists of three or more plies whose individual fiber orientations are obliquely disposed with respect to each other, in addition to the normal lazy tong effects of cross drafting, the "serpentine effect" may also be obtained. It is thus possible to produce laterally extensible fabrics which expand on the lazy tongs principle but which are inherently stronger and more resistant to

tear than the laterally extensible fabrics produced by the serpentine effect alone.

In carrying the invention into practice the conventional binder media and island bonding operations of the prior art may be used. Typical procedures and binder media of the general type applicable to the practice of the present invention include those disclosed in the Joshua Goldman Patent 2,039,312 or in the Joseph Goldman Patent 2,407,548 or in the Esther Goldman Patent 2,545,952. Such operations and media, being well known and conventional, need not be described herein, since reference may readily be made to the prior art including the patents mentioned.

I prefer to use island bonding wherein the lateral surface covered by the binder areas does not substantially exceed about 35% of the total lateral surface of the web. This condition insures attainment of lateral extensibility and also desirable textile-like properties of softness, drape and loft. However some of the advantages of the invention may be attained to a degree with line bonding. For example, the di- or tri-oriented webs may be bonded by imprinting thereon a diamond grid binder pattern consisting of two series of parallel continuous lines of binder extending obliquely across the web at substantially the same angles of inclination as the angles of orientation of the plies of the base web. Island bonding, however, is preferable, particularly the type of island bonding illustrated in the drawings herein.

After the bonding operation, the bonded fabric may be cross drafted to expand the fabric on the lazy tongs principle. Such cross drafting produces a "peach fuzz effect" from non-oriented fibers, especially those lying in a direction substantially parallel to the horizontal axis of the lazy tong parallelograms. In addition, as mentioned above, in the case of the tri-oriented webs, cross drafting produces the serpentine effect if the discrete binder areas are arranged in parallel, overlapping columns that are parallel to one of the three axes of fiber orientation of the three ply base web.

After cross drafting, the laterally extended fabric may be used as such, if desired, or it may be rebonded, following in general the process described above in connection with the manufacture of a pseudo-isotropic fabric. Since the cross strength of the unextended, "polyoriented" fabric is greater than an otherwise identical fabric wherein the fibers are substantially oriented in a single direction, the amount of cross drafting before rebonding that is necessary to reverse the normal long to cross tensile strength ratio is correspondingly reduced.

The cross drafted product of the present invention, either before or after rebonding, may be plied with an unbonded web of either singly or polyoriented fibers, to produce a laminated structure that can be bonded together to form a product corresponding to the above mentioned "pseudo cross lay". If desired, of course, the bonded polyoriented web of the present invention, in either its extended or unextended condition, may be laminated with other fabrics or materials, such as a non-woven fabric of the same or different structure or design.

The term "polyoriented" as used herein is understood to include the di-oriented as well as the tri-oriented webs and the fabrics made therefrom. The term "textile fibers" includes fibers of any type that are as long as the conventional textile fibers which are capable of being spun into yarn and woven into cloth. Generally speaking, this includes fibers whose average length is about one-half inch or longer.

Having now described my invention in detail and illustrated the preferred manner in which it may be carried into practice, it will be readily apparent to those skilled in the art that many variations, applications, modifications and extensions of the basic principles involved may be made without departing from its spirit or scope. Thus, for example, although I have illustrated the invention in connection with di- and tri-oriented webs (both of which I term "polyoriented"), it is apparent that the principles involved are applicable to webs made from more than three plies, each oriented obliquely with respect to the others. I therefore intend to be limited only in accordance with the appended patent claims.

I claim:

1. A nonwoven fabric comprising a bonded web composed of at least two plies of oriented textile fibers, the directions of orientation of the respective plies being inclined obliquely with respect to each other.

2. A nonwoven fabric comprising an island bonded web composed of at least two plies of oriented textile fibers whose directions of fiber orientation are obliquely disposed with respect to each other, said fabric being characterized by high capacity for extension on the lazy tongs principle when subjected to extensional stress in a direction generally transverse to the fiber orientations of said plies.

3. A nonwoven fabric comprising a web composed of at least two plies of oriented textile fibers whose directions of fiber orientation are obliquely disposed with respect to each other, said web being bonded into a self-sustaining fabric by a multiplicity of discrete areas of binder adapted to coat with the fibers in said plies to form a plurality of interconnected, geometric figures that are collapsible when the web is subjected to extensional stress in a direction generally transverse to the fiber orientations of said plies.

4. A nonwoven fabric comprising a web composed of at least two plies of oriented textile fibers whose directions of fiber orientation are obliquely disposed with respect to each other, said web being bonded into a self-sustaining fabric by a multiplicity of discrete areas of binder infused locally into the body of the web and adapted to form with the oriented fibers in each of said plies a plurality of interconnected, collapsible polygons whose pivotal points are formed by said binder areas and whose sides are formed by bundles of substantially parallel fibers connecting said binder areas.

5. A nonwoven fabric comprising a web composed of at least two plies of oriented textile fibers whose directions of fiber orientation are obliquely disposed with respect to each other, said web being bonded into a self-sustaining fabric by a multiplicity of discrete areas of binder infused locally into the body of the web and adapted to form with the oriented fibers in the respective plies at least two series of parallel, substantially straight, obliquely disposed fiber bands, the bands of one parallel series intersecting the bands of the other parallel series, said binder areas being located at the points of intersection of said bands.

6. A non-woven fabric having a reticular structure and comprising two series of parallel, substantially straight bands of textile fibers, the bands of the two parallel series being disposed in different but parallel planes and at an oblique intersecting angle with respect to each other, said bands being united together by discrete areas of binder locally infused into the body of both series of bands at their overlying angles of intersection.

7. The fabric of claim 6 wherein each of said bands comprises a multiplicity of substantially parallelized, unspun textile fibers.

8. The fabric of claim 6 wherein a multiplicity of substantially parallelized, unspun textile fibers is disposed between, and substantially oriented with, each of said bands in each of said series.

9. A non-woven fabric having a reticular structure and comprising two series of parallel, substantially straight bands of fibers, the bands of each series being disposed in different but parallel planes, each band in each series comprising a multiplicity of substantially parallelized unspun textile fibers, the bands of one parallel series overlying and being obliquely inclined with respect to the bands of the other parallel series and being united together by discrete areas of binder infused locally into the body of both bands at their overlying points of intersection, said bands coating with said binder areas to form a multiplicity of interconnecting parallelograms that are collapsible on the lazy tongs principle when the fabric is subjected to extensional stress in a direction parallel to either diagonals of said parallelograms.

10. The fabric of claim 9 wherein a multiplicity of substantially parallelized unspun textile fibers is disposed between, and substantially oriented with, each of said bands in each of said series.

11. A method which comprises plying at least two webs of substantially oriented textile fibers, with their respective orientation directions obliquely disposed with respect to each other, whereby to form a composite web having two primary directions of fiber orientation that are oblique to each other; and then bonding said composite web to convert it into a self-sustaining nonwoven fabric.

12. A method which comprises plying at least two webs of substantially oriented textile fibers, with their

respective axes of orientation obliquely disposed with respect to each other, whereby to form a composite web having two primary directions of fiber orientation that are oblique to each other; and then converting said composite web into an island bonded fabric.

13. The method of claim 12 wherein said binder pattern covers not substantially more than about 35% of the lateral surface of the web.

14. The method of claim 12 wherein said fabric is then cross drafted, in order to expand said fabric on the lazy tongs principle and to effect a uniform reorientation of a substantial proportion of the fibers oriented in either of said primary orientation directions.

15. The method of claim 12 wherein said fabric is cross drafted in order to expand said fabric on the lazy tongs principle and effect uniform reorientation of a substantial proportion of the fibers oriented in either of said primary orientation directions; and the cross drafted fabric is then dimensionally stabilized in its expanded state.

16. A method which comprises plying at least two webs of substantially oriented textile fiber with their respective primary orientation directions obliquely disposed with respect to each other; converting said plied webs into an island bonded fabric by bonding the same with a discontinuous binder pattern uniformly disposed over not more than 35% of the lateral surface of said plied webs; cross drafting the island bonded fabric in order to expand the same on the lazy tongs principle with substantially uniform reorientation of fibers originally oriented in either of said primary orientation directions; and then rebonding the cross drafted fabric to dimensionally stabilize said fibers in their reoriented condition.

17. A method which comprises continuously forming at least two separate webs of substantially parallelized or oriented textile fibers, the webs being of substantially equal

width and moving along separate paths whose axes are laterally displaced from, but converging toward, each other at an oblique angle; bringing said converging web into face-to-face relationship, with one web overlying the other with their corresponding edges in substantial alignment to form a composite laminated web comprising at least two plies whose primary orientations are obliquely disposed with respect to each other; converting the composite web into an island bonded fabric by bonding the web with a discontinuous binder pattern covering not substantially more than about 35% of the total lateral surface of the web; cross drafting the island bonded fabric after the binder pattern thereof has set, in order to effect further reorientation of the fibers, and then dimensionally stabilizing the cross drafted fabric by rebonding the cross drafted fabric.

#### References Cited in the file of this patent

#### UNITED STATES PATENTS

|    |           |              |                |
|----|-----------|--------------|----------------|
| 20 | 1,507,949 | Angier       | Sept. 9, 1924  |
|    | 1,831,403 | Woodward     | Nov. 10, 1931  |
|    | 2,039,312 | Goldman      | May 5, 1936    |
|    | 2,055,410 | Hurst et al. | Sept. 22, 1936 |
|    | 2,407,548 | Goldman      | Sept. 10, 1946 |
|    | 2,407,949 | Gurwick      | Sept. 10, 1946 |
|    | 2,498,197 | Baxter       | Feb. 21, 1950  |
|    | 2,514,108 | Vogt         | July 4, 1950   |
|    | 2,523,860 | Budden       | Sept. 26, 1950 |
|    | 2,545,952 | Goldman      | Mar. 20, 1951  |
|    | 2,550,686 | Goldman      | May 1, 1951    |
|    | 2,574,221 | Modigliani   | Nov. 6, 1951   |

#### FOREIGN PATENTS

|               |               |
|---------------|---------------|
| Great Britain | Nov. 12, 1942 |
| Belgium       | Dec. 30, 1950 |